

(No Model.)

2 Sheets—Sheet 1.

J. D. FRANCKS.

Process for Preserving Wood.

No. 231,419.

Fig. 1. Patented Aug. 24, 1880.



Fig. 2.



Fig. 3.



Attest:

R. F. Barnes.  
Warren S. Sely

Inventor:

J. D. Francks  
by Ellis Spear  
Attest

(No Model.)

2 Sheets—Sheet 2.

J. D. FRANCKS.

Process for Preserving Wood.

No. 231,419.

Patented Aug. 24, 1880.

Fig. 4.



Fig. 5.



Fig. 6.



Attest:

R. F. Barnes.  
Warren Seely.

Inventor:

J. D. Francks  
by Elie Spear  
Atty

# UNITED STATES PATENT OFFICE.

JONAS D. FRANCKS, OF HANOVER, GERMANY.

## PROCESS FOR PRESERVING WOOD.

SPECIFICATION forming part of Letters Patent No. 231,419, dated August 24, 1880.

Application filed April 27, 1880. (No model.) Patented in Germany January 20, 1880.

To all whom it may concern:

Be it known that I, JONAS D. FRANCKS, of Hanover, Germany, have invented an Improved Process for Treating Wood, of which 55  
5 the following is a specification.

My invention relates to the treatment of wood for the purpose of increasing its durability and the beauty of its appearance.

It consists, essentially, in impregnating the 10 wood with a mixture of lime-water and urine. This mixture, applied to the wood in the manner hereinafter described, greatly increases the density and solidity of all kinds of wood, and at the same time thoroughly changes and 15 improves the original tint, thereby greatly increasing the durability and beauty of the wood, whatever the variety to which it may be applied.

The mixture specified above may be applied to the wood in any of the ways or by means 20 of any of the appliances used for like purposes.

It is only necessary, first, that the acids and resins contained naturally in the wood should be expelled, and that the wood thus freed from these substances should be saturated with the 25 described mixture.

I have shown two forms of apparatus adapted to effect the saturation of any kind of wood according to my invention.

On Sheet 1 the three figures represent a 30 form of apparatus adapted to be moved readily from place to place and more elaborate in structure. In these figures a receptacle, A, is shown, adapted to receive the wood and to be closed tightly by a cover, a.

After the wood 35 has been so inclosed steam is let on through the pipe d at a pressure of about two atmospheres. The application of the steam should be continued long enough to extract from the wood the acids, juices, and resins specified 40 above.

The length of time required for this purpose will vary greatly with the variations in the thickness or kinds of wood. After these substances have been removed by the application of the steam the alkaline liquid or lye 45 is admitted in a heated condition, by cock, e, into the mixture-receptacle, which contains a mixture of lime-water and urine in about equal proportions. The cock e is now shut, the air is exhausted from the receptacle A by means 50 of the air-pump B. The cock f is then opened, and in a short time the wood within the recep-

tacle will have absorbed the mixture thus admitted. The air-pump is then stopped, the cock f shut, and the forcing-pump C put into operation, by means of which a further supply 55 of mixture is forced into the receptacle up to a pressure of from one to four atmospheres.

The amount of pressure and the length of time during which it is maintained must depend upon the quality of the different species of 60 wood under treatment and the form or thickness of the wood. In like manner the application of the whole process must in practice be varied in accordance with the qualities required of the article to be manufactured, 65 whether it be desired to harden the wood and increase its density throughout its whole thickness or only upon the surface. The pressure may be kept up to the height stated for eight, twelve, or twenty-four hours, or even 70 longer; but when the woods have been sufficiently treated for the purpose for which they are required they are cooled down, the mixture is turned off into some special receptacle, and the woods are taken from the receptacle A, having 75 been rendered more dense, harder, and having been permanently improved in their tints. They may then be cleaned and treated in accordance with the use for which they are intended, or may be piled up for drying, which 80 will speedily take place.

The cost of preparing woods by this process is very slight. For deals of one inch in thickness the cost is about two German pfennigs per square foot. 85

The device shown in Sheet 2 is more simple, consisting of a simple tank or reservoir suited to receive the wood and the mixture, with a grate underneath for the direct application of a fire to the bottom. 90

With this apparatus the boiling must be kept up from one to four days, according to the quality of the wood or the thoroughness of the action of the mixture thereupon, and during this time fresh supplies of the mixture should be added at proper intervals in order to obtain a good result. The result of increased density and solidity will be apparent, even before the woods are dry, upon sawing them across at the ends, the effect being shown by the depth 100 of the change in the tint, but when the woods are dried the effect is more marked in the in-

creased density and hardness. Wood thus treated is proof against the wood-worm and fungus, the density preventing the penetration of moisture. It is also rendered less combustible, more elastic, and capable of receiving better polish, and even pine woods thus treated would not require paint in order to give them the tint and appearance of hard woods. Other advantages in woods thus treated are that they are not subject to shrinkage and are more readily dried than wood in its natural condition.

Having thus described my invention, what I claim is—

The described process of treating wood, consisting in saturating the same with a mixture of lime-water and urine in a heated state, substantially as described.

In testimony whereof I have signed my name to this specification in the presence of two subscribing witnesses.

J. D. FRANCKS.

Witnesses:

WILLIAMS C. FOX,  
JONIS. KRACKE.